

# UNITED STATES PATENT OFFICE.

JOHN T. COUSE, OF COCHRAN, GEORGIA.

## ROOFING COMPOUND.

981,916.

No Drawing.

Specification of Letters Patent. Patented Jan. 17, 1911.

Application filed January 25, 1909. Serial No. 474,126.

*To all whom it may concern:*

Be it known that I, JOHN T. COUSE, citizen of the United States, residing at Cochran, in the county of Pulaski and State of Georgia, have invented certain new and useful Improvements in Roofing Compounds, of which the following is a specification.

This invention comprehends certain new and useful improvements in waterproofing compounds for roofing or the like, and the invention has for its object an improved compound that is susceptible of being easily and cheaply prepared, and that is designed to be applied to a foundation or structural 10 ply of felt or other roofing fabric, to provide a composition shingle to supersede the ordinary wooden shingle, and capable of 15 withstanding the erosive effect of the weather. And a further object of the invention is an improved composition which is colored as desired, so as to impart a pleasing effect to the shingle and effect a material 20 economy in the time, labor and expense involved in painting the ordinary shingle.

In carrying out my invention, I prepare 25 a mixture of the following ingredients which are combined in substantially the proportions specified, viz: sifted sand, 70 lbs.; Portland cement, 25 lbs.; graphite 10 lbs. These ingredients are agitated to effect 30 the thorough mixture thereof. In order to impart the desired color to the compound, 5 lbs. of mineral pigment are added to the above mixture. This mixture is then introduced into and incorporated with 5 gallons 35 of liquid asphaltum, so as to complete the preparation of the waterproofing compound which is initially of a plastic nature.

In the practical use of my improved compound for manufacturing shingles or the like, I take a structural ply or foundation 40 of felt which is cut into the desired size and shape, and which is impregnated with the plastic compound, with the coating or 45 layer of the compound on one or both sides of the ply, tapering toward one end of the same in more perfect imitation of the ordinary wooden shingle, and for a purpose that will be obvious. After exposure to the 50 atmosphere for a certain period, the plastic coating becomes very hard, so as to be capable, when the shingle is applied to the building, of withstanding the erosive effect

of the weather and the weight of snow or the like accumulated upon the roof. The liquid 55 asphaltum penetrates the fabric and renders the latter water proof, while the more solid particles form a hard exterior coating for the fabric. The presence of the graphite in the compound also prevents the 60 rays of the sun from injuriously affecting the asphaltum.

It is to be understood that it is not necessary to use a foundation of felt, but any suitable roofing fabric could be employed, 65 as for instance, cloth, fibrous-board, perforated metal, or screening, said structural ply being preferably provided with nail holes before the compound is applied thereto. Attention is also directed to the fact 70 that this compound may be easily and cheaply manufactured; that it is entirely waterproof, and that the foundation ply may be impregnated therewith without the 75 application of heat.

It has been found, after repeated experiments, that by combining the several ingredients in the specific proportions stated, a composition shingle or roofing slab is produced having a hard exterior surface 80 which is not affected by the rays of the sun, and which will effectually withstand the deleterious action of the elements for an indefinite period without disintegrating.

Having thus described the invention, what 85 I claim is:

1. The herein described composition of matter for saturating and coating roofing fabric, consisting of sifted sand 70 lbs., Portland cement 25 lbs. and graphite 10 lbs., the 90 parts being incorporated with 5 gallons of liquid asphaltum.

2. The herein described composition of matter for saturating and coating roofing fabric, consisting of sifted sand 70 lbs., Portland cement 25 lbs., graphite 10 lbs. and mineral pigment 5 lbs., the parts being 95 incorporated with 5 gallons of liquid asphaltum.

In testimony whereof I affix my signature 100 in presence of two witnesses.

JOHN T. COUSE.

Witnesses:

J. N. WYNNE,  
L. M. NE SMITH.